

Feb. 19, 1924.

1,484,569

J. F. SCHEID

CERAMIC BODY

Filed Aug. 24, 1921

Fig. 1



Fig. 2



Inventor:  
Johannes Friedrich Scheid  
by A. K. Lueder  
Attorney

## UNITED STATES PATENT OFFICE.

JOHANNES FRIEDRICH SCHEID, OF MARGARETHENHUTTE, GROSSDUBRAU, GERMANY,  
ASSIGNOR TO THE FIRM: H. SCHOMBURG & SÖHNE, OF MARGARETHENHUTTE,  
GROSSDUBRAU, GERMANY.

## CERAMIC BODY.

Application filed August 24, 1921. Serial No. 494,968.

To all whom it may concern:

Be it known that I, JOHANNES FRIEDRICH SCHEID, a citizen of Germany, residing at Margarethenhutte, Grossdubrau, Saxony, Germany, have invented certain new and useful Improvements in Ceramic Bodies (for which I have filed applications in Germany, July 29, 1914; Austria, June 7, 1916; Czechoslovakia, July 19, 1919; Yugoslavia, 10 June 4, 1921), of which the following is a specification.

My invention relates to a method of securing a body of ceramic material in a hollow body of a like material and in particular to the manufacture of insulators consisting of two or more parts.

Insulators for high potentials cannot be manufactured in one part, as it is not possible to manufacture objects of porcelain having high dielectric strength beyond a certain wall thickness. In the manufacture of suspension insulators, in which a connection of several parts by simply cementing them into one another, does not reliably prevent 20 the inner part from becoming loose and falling out, it has been attempted to obtain a greater mechanical strength by utilizing the shrinking of porcelain when being dried and baked. Porcelain has a shrinkage from 25 the crude condition up to the condition of white dryness of about 5 to 6 per cent and from this condition to the finished baked condition of 10 to 12 per cent. It has been proposed to make the inner part of the insulator conical and to insert it in a correspondingly conical hollow space of the insulator body. The inner part is then dried and, in this condition, introduced into the 30 hollow body which is still moist. After 35 drying, the hollow body is expected to shrink to such an extent, that the inner part can no more fall out. Whereupon both parts are baked together. The dimensions are such, that in the finished insulator there 40 is an interstice between the hollow body and the inner part which is filled with cement. In this method the hollow body projects over the inner part only very little as it shrinks but little in drying.

According to my invention, far more projection and considerably greater mechanical strength are obtained by first baking the inner part, thereupon inserting it in the hol-

low body which has only been dried, and then baking the hollow body. 55

My improved method can be used in the manufacture of insulators consisting of a plurality of parts as well as for the securing of insulator supports in suspension insulators. 60

In the drawings affixed to this specification and forming part thereof, two embodiments of my invention are illustrated by way of example. In the drawings—

Fig. 1 is an elevation partly in section of 65 an insulator consisting of two parts and

Fig. 2 a similar view illustrating a method of securing an insulator support in a suspension insulator.

Referring to Fig. 1, the inner part 1 of an 70 insulator consisting of two parts has a spherical head 2 at its upper end. The hollow space of the body 3 is so formed that when the body has been baked, it will surround the inner section on all sides with a 75 clearance of about 2 mm. In the example illustrated the radius  $a$  of the head 2 in its baked condition is 29 mm. The narrowest portion  $b$  of the hollow space of the body has a radius of about 30 mm. in unbaked 80 condition, so that it is possible to introduce the head 2 into it. After baking, however, the radius of the hollow space at  $b$  is only about 26 mm., so that the head 2 can not be withdrawn. If now a layer of cement 4 is 85 inserted between the body and the inner part, it will be placed under a compression stress at  $c$ , when a pull is exerted on part 1. Obviously, the part 1, instead of having a single head 2, might also have a plurality 90 of corrugations or the like, the wall of the hollow body being shaped in conformity and with a slight clearance.

Fig. 2 illustrates the application of my invention to the securing and support of the 95 insulator pin in the hollow space of the body. Here a ball 5 of porcelain which is provided with a hole at 6 and flattened at 7 is baked and inserted in the hollow space of a body 3 which is not yet baked, the dimensions of the body being, as before, such that when baked, it will shrink to a diameter at 100 its narrowest portion which is less than the diameter of the ball. After baking the body, the ball 5 is turned until its flattened 105 face 7 is directed downward and a nut 8

is placed on it so as to complete the shape of the ball. The ball is now again turned in the hollow space together with the nut, so that the nut is on top of the ball (Fig. 2) and the pin 9 is inserted through the hole 6 and screwed into the nut. Finally, the space between the pin and the hollow body 3 is filled with cement. When a pull is exerted on the pin, the cement will be placed under a compression stress at c.

In manufacturing insulators consisting of more than two parts, the method first described is repeatedly applied. The method last described can also be used for securing the pin in insulators consisting of two or

more sections.

I claim:

1. The method of fixing in a hollow of a ceramic body a second ceramic body of greater width than the opening of the said hollow, consisting in introducing said second body in baked condition in the hollow of

said first ceramic body while this latter is still in a raw state and before it has been subjected to heat treatment.

25

2. The method which consists in introducing in the hollow of an unbaked ceramic body a perforated baked ceramic ball-shaped body with a flat face, baking said hollow body, placing a nut on the flat face of said ball shaped body, turning said body and nut and inserting a screw-bolt.

30

3. In a ceramic insulator in combination, a hollow ceramic body, a perforated ball-shaped ceramic body in the hollow of said body, said perforated body being of greater width than the opening of said hollow body, a nut intermediate said ball-shaped body and the wall of said hollow body and a screw-threaded support extending through 35 said ball-shaped body and said nut.

40

In testimony whereof I affix my signature.

JOHANNES FRIEDRICH SCHEID.